

## UNITED STATES PATENT OFFICE

2,374,183

## SILVER SOLDER

George Durst, Attleboro, Mass., assignor to Metals & Controls Corporation, Attleboro, Mass., a corporation of Massachusetts

No Drawing. Application October 9, 1943,  
Serial No. 505,668

9 Claims. (Cl. 75—173)

This invention relates to silver solder, and with regard to certain more specific features to low-temperature-flowing silver solder.

Among the several objects of the invention may be noted the provision of a low-cost, easily-manipulated silver solder, or what may be called a silver brazing alloy, of low-temperature-flowing characteristics; the provision of a solder of the class described which has a high capillarity and thus a high wetting or spreading characteristic on metal surfaces to which it is applied; and the provision of a solder of this class which has sufficient ductility for cold working. Other objects will be in part obvious and in part pointed out hereinafter.

The invention accordingly comprises the elements and combinations of elements, the proportions thereof, and features of composition, which will be exemplified in the substances and products hereinafter described, and the scope of the application of which will be indicated in the following claims.

One of the best-known easy-flowing silver solders is composed of silver, copper, zinc and cadmium, in proportions which are presumably close to being a quaternary eutectic. They have a spreading temperature of about 1175° F. to 1180° F. An example of this old solder is (% by weight):

(I)

|         |      |
|---------|------|
| Silver  | 50.0 |
| Copper  | 15.5 |
| Zinc    | 16.5 |
| Cadmium | 18.0 |

This is a solid at 1160° F. and completely liquid at 1175° F. The free spreading temperature is about 1175° F. to 1180° F., depending upon the character of the receiving surface.

The present invention reduces the temperature of spreading while very greatly increasing the spreading effect itself of solders of the above class.

Following is a table of component proportions of three examples (II), (III) and (IV), of my new solder, given in percentage weights:

|         | (II) | (III) | (IV) |
|---------|------|-------|------|
| Silver  | 45.0 | 46.0  | 45.0 |
| Copper  | 17.5 | 17.0  | 17.0 |
| Zinc    | 16.5 | 16.5  | 16.5 |
| Cadmium | 19.7 | 19.5  | 20.5 |
| Tin     | 0.5  | 0.5   | 0.5  |
| Lead    | 0.8  | 0.5   | 0.5  |

The above alloys have a spreading temperature of approximately 1150—1155° F., which is much lower as compared to the above-mentioned spreading temperature of 1175° F. to 1180° F. A given amount of the new solder will spread about twice as much in area on copper. It solidifies at about 1135° F. Its ductility in cold working is comparable to that of the described old solder.

The importance of the additions of tin and lead, as compared to possible additions of other materials which might suggest themselves, such as gallium, indium, antimony, thallium, and bismuth, is that indium and gallium are too expensive while the other metals mentioned cause excessive embrittlement.

The small additions of tin and lead, while substantially reducing temperature of spreading and increasing the spreading activity itself, do not excessively reduce the ductility in cold working.

To gain advantages along the above-described lines for solder it has been suggested that the easy-flowing type of solder have introduced therein small additions of lithium or sodium or the like, but alkali metals such as these are expensive, difficult to handle, and in general are used in silver solders having a higher melting range from those herein contemplated.

Suitable useful ranges of proportions for the invention are as follows, wherein the combined zinc and cadmium contents should not exceed 40%, all by weight:

|               | (V)     | Per cent |
|---------------|---------|----------|
| Silver        | 40—50   |          |
| Copper        | 15—19   |          |
| Zinc          | 14—20   |          |
| Cadmium       | 18—24   |          |
| Tin plus lead | 0.1—5.0 |          |

I have obtained satisfactory results with lead only according to the following two ratios by per cent weight:

|         | (VI) | (VII) |
|---------|------|-------|
| Silver  | 50   | 45    |
| Copper  | 16   | 16    |
| Zinc    | 16   | 16    |
| Cadmium | 15   | 21    |
| Lead    | 3    | 2     |

The additions of both tin and lead are however preferable with regard to wetting characteristics.

In view of the above, it will be seen that the several objects of the invention are achieved and other advantageous results attained.

As many changes could be made in the above alloy and solder product, without departing from the scope of the invention, it is intended that all matter contained in the above description shall be interpreted as illustrative and not in a limiting sense.

I claim:

1. A low-flow-temperature silver solder comprising approximately by weight, 40-50% of silver; 15-19% of copper; 14-20% of zinc; 18-24% of cadmium; and 0.1-5.0% total of tin and lead.

2. A low-flow-temperature silver solder comprising approximately by weight 40-50% of silver; 15-19% of copper; 14-20% of zinc; 18-24% of cadmium and 0.1-5.0% of lead.

3. A low-flow-temperature silver solder having a high wetting activity, comprising approximately by weight 40-50% silver; 15-19% copper; 14-20% zinc; 18-24% cadmium; the combined contents of zinc and cadmium not to exceed approximately by weight 40%; and small amounts of tin and lead, not to exceed a total of approximately by weight from 0.1-5.0%.

4. A low-flow-temperature silver solder having a high wetting capacity comprising approximately by weight the following proportions; sil-

ver, 45%; copper, 17.5%; zinc, 16.5%; cadmium, 19.7%; tin, 0.5%; and lead, 0.8%.

5. A low-flow-temperature silver solder having a high wetting activity comprising approximately by weight, silver, 46%; copper, 17%; zinc, 16.5%; cadmium, 19.5%; tin, 0.5%; and lead, 0.5%.

6. A low-flow-temperature silver solder having a high wetting activity comprising approximately by weight, silver, 45%; copper, 17%; zinc, 16.5%; cadmium, 20.5%; tin, 0.5%; and lead, 0.5%.

7. A low-flow-temperature silver solder having a high wetting capacity comprising approximately by weight the following proportions; silver, 45-50%; copper, 16%; zinc, 16%; cadmium, 15-21%; and lead, 3-2%.

8. A low-flow-temperature silver solder having a high wetting capacity comprising approximately by weight 50% silver; 16% copper; 16% zinc; 15% cadmium; and lead 3%.

9. A low-flow-temperature silver solder having a high wetting capacity comprising approximately by weight the following proportions; silver, 45%; copper, 16%; zinc, 16%; cadmium, 21%; and lead, 2%.

GEORGE DURST.